



US005998122A

# United States Patent [19]

Spara et al.

[11] Patent Number: 5,998,122

[45] Date of Patent: Dec. 7, 1999

[54] **PHOTOGRAPHIC ELEMENT CONTAINING PYRAZOLOAZOLE MAGENTA COUPLER AND A SPECIFIC ANTI-FADING AGENT**

[75] Inventors: **Paul P. Spara; Stanley W. Cowan**, both of Rochester, N.Y.

[73] Assignee: **Eastman Kodak Company**, Rochester, N.Y.

[21] Appl. No.: **09/134,567**

[22] Filed: **Aug. 14, 1998**

[51] Int. Cl.<sup>6</sup> ..... **G03C 1/08**; G03C 7/26; G03C 7/32

[52] U.S. Cl. ..... **430/551**; 430/558

[58] Field of Search ..... 430/551, 558

## [56] References Cited

### U.S. PATENT DOCUMENTS

|           |         |                  |       |         |
|-----------|---------|------------------|-------|---------|
| 5,017,465 | 5/1991  | Nishijima        | ..... | 430/551 |
| 5,082,766 | 1/1992  | Nishijima et al. | ..... | 430/551 |
| 5,104,782 | 4/1992  | Seto et al.      | ..... | 430/551 |
| 5,236,819 | 8/1993  | Kadokura et al.  | ..... | 430/551 |
| 5,352,573 | 10/1994 | Seto et al.      | ..... | 430/551 |
| 5,415,989 | 5/1995  | Wolff            | ..... | 430/523 |
| 5,561,037 | 10/1996 | Jain et al.      | ..... | 430/551 |

Primary Examiner—Geraldine Letscher  
Attorney, Agent, or Firm—Arthur E. Kluegel

## [57] ABSTRACT

The disclosure describes a photographic element comprising a light sensitive silver halide emulsion layer having associated therewith a magenta dye forming coupler containing an azole nucleus and a ballasted compound having Formula I,



wherein

each R<sub>1</sub> is independently selected from the group consisting of hydrogen and an alkyl, aryl, acyl and acylamino group;

L represents a linking atom or group bonded to the phenyl ring by a heteroatom;

each "a" independently represents a substituent group at least one of which is linked to the phenyl ring by an N, S, C or O atom and q is 1 to 5;

provided that the selection of L and the "a" groups results in no more than one oxygen bond to the phenyl ring.

**17 Claims, No Drawings**

**PHOTOGRAPHIC ELEMENT CONTAINING  
PYRAZOLOAZOLE MAGENTA COUPLER  
AND A SPECIFIC ANTI-FADING AGENT**

**FIELD OF THE INVENTION**

This invention relates to photographic elements containing a light sensitive silver halide emulsion layer having associated therewith a magenta dye forming coupler and a phenyl compound bearing a certain alcoholic group.

**BACKGROUND OF THE INVENTION**

In a silver halide photographic element, a color image is formed when the element is exposed to light and then subjected to color development with a primary aromatic amine developer. Color development results in imagewise reduction of silver halide and production of oxidized developer. Oxidized developer reacts with one or more incorporated dye-forming couplers to form an imagewise distribution of dye.

The dyes that are formed by any color coupler during processing have a tendency to fade over time as a result of exposure to light, heat and humidity. As all three image dyes of a typical color element fade, this results in overall fading of the image over time. Since the three image dyes may not fade at the same rate, an apparent change in image color may result. Such change is particularly noticeable in the case of magenta image dye fading.

A variety of magenta dye-forming coupler types have been used in photographic materials. Among the known magenta dye-forming couplers are cyclic azoles such as pyrazolotriazoles, pyrazolobenzimidazoles, and imidazopyrazoles. These couplers contain bridgehead nitrogen 5,5 fused ring systems and include such couplers as pyrrolo[1,2-b]pyrazoles, pyrazolo[3,2-c][1,2,4]triazoles, pyrazolo[2,3-b][1,2,4]triazoles, imidazo[1,2-b]pyrazoles, imidazo[1,5-b]pyrazoles, imidazo[1,2-a]imidazoles, imidazo[1,2-b][1,2,4]triazoles, imidazo[2,1-c][1,2,4]triazoles, imidazo[5,1-c][1,2,4]triazoles and [1,2,4]triazolo[3,4-c][1,2,4]triazole. Also included are 5,5,6 fused ring systems that include such couplers as pyrazolo[3,2-6]bicycloimidazoles.

A significant disadvantage of pyrazolozole couplers is fading of the image dyes formed upon photographic processing due to extended exposure to low levels of light. Compounds which are included in photographic elements to reduce image dye fading are known as stabilizers or anti-fade agents. Inclusion of stabilizers in color photographic materials can reduce the deterioration of the dye images which occur over time as a result of the action of light, heat or humidity. This is true for dyes formed from pyrazolozole couplers. U.S. Pat. Nos. 5,236,819, 5,561,037, and 5,082,766 and German Published Patent Application OLS 4,307,194 describe the use of certain stabilizers with pyrazolozole couplers to improve their dye stability. However, it is desirable to further improve the light stability of dyes derived from azole magenta dye forming couplers, and thus retain the color rendition of the image for a longer period of time.

A problem to be solved is to provide a photographic element that will yield magenta dye images that have low fading when exposed to light.

**SUMMARY OF THE INVENTION**

The invention provides a photographic element comprising a light sensitive silver halide emulsion layer having associated therewith a magenta dye forming coupler con-

taining an azole nucleus and a ballasted compound having Formula I,



wherein

each R<sub>1</sub> is independently selected from the group consisting of hydrogen and an alkyl, aryl, acyl and acylamino group;

L represents a linking atom or group bonded to the phenyl ring by a heteroatom;

each "a" independently represents a substituent group at least one of which is linked to the phenyl ring by an N, S, C or O atom and q is 1 to 5;

provided that the selection of L and the "a" groups results in no more than one oxygen bond to the phenyl ring.

Photographic elements of the present invention yield magenta dye images that have low fading when exposed to light.

**DETAILED DESCRIPTION OF THE INVENTION**

A formula for compound I is represented by Formula I,



wherein

each R<sub>1</sub> is independently selected from the group consisting of hydrogen and an alkyl, aryl, acyl and acylamino group;

L represents a linking atom or group bonded to the phenyl ring by a heteroatom;

each "a" independently represents a substituent group at least one of which is linked to the phenyl ring by an N, S, C or O atom and q is 1 to 5;

provided that the selection of L and the "a" groups results in no more than one oxygen bond to the phenyl ring.

L is any group suitable for linking the ethoxy substituent to the phenyl ring through a heteroatom or group. Examples include —O—, —OP(O)(OR)O—, —CONR—, —NRCO—, —NRSO<sub>2</sub>—, —SO<sub>2</sub>NR—, and —SO<sub>2</sub>—, in which R is an alkyl or aryl group. L may also include such groups having alkylene, arylene, or hetero groups such as ether groups in the group L.

The group(s) "a" may be any substituent group. Substituent groups may be any of the groups defined hereinafter. There is present at least one "a" group that is bonded to the phenyl ring by an N, S, C or O atom, provided that the selection of L and the "a" groups results in no more than one oxygen bond to the phenyl ring. Particularly suitable is an "a" group where the link to the phenyl ring is —NHSO<sub>2</sub>—. An example is:



5

10

15

20

25

30

35

40

45

50

55

60

65

-continued



wherein:  $R_1$  and  $R_2$  are alkyl groups having a total of 9-30 carbon atoms.

More specifically, the following compound is useful.



**5**

-continued



**7**

-continued

**8**

-continued

I-21

5



I-22

10



I-23

15



I-24

20



I-25

25



I-26

30



I-27

35



I-28

40



I-29

45



I-30

50



I-31

55



60



65

65

**9**

-continued



I-32

5



I-33 15



I-34 25

30

35

We have found that highly stable magenta dye images formed from azole magenta couplers can be obtained if there is associated with the coupler a combination of stabilizer compounds I and S, shown below, and more suitably a combination of stabilizer compounds I, S, and R, shown below.

Formula S is as follows:



wherein:

R<sub>3</sub> represents an aryl group or a heterocyclic group;

Z<sub>1</sub> and Z<sub>2</sub> each represent an alkylene group having 1 to 3 carbon atoms provided that the total number of carbon atoms in the ring is 3 to 6; and

n is an integer of 1 or 2;

The stabilizers that have the Formula S are believed to stabilize by acting as singlet oxygen quenchers. In this formula the aryl and heterocyclic group represented by R<sub>3</sub> include phenyl, 1-naphthyl, 2-furyl and 2-thienyl groups. They can be substituted with groups described hereinafter for Formula III for R<sub>6</sub>, as can be the alkylene groups represented by Z<sub>1</sub> and Z<sub>2</sub>.

Preferred stabilizers represented by Formula S, are those having the following Formula S1:

**10**

wherein:

R<sub>8</sub> represents halogen or alkyl, alkoxy, alkylthio, amido, or ureido groups;

R<sub>9</sub> is alkyl;

r is an integer of 1 or 2; and

s is an integer of 0 to 4.

Representative examples of stabilizer having Formula S are:



S-1



S-2



S-3



S-4



S-5



S-6



S-7



S-8

Formula R is as follows:



R

5

wherein:

- each  $R_1$  independently represents a hydrogen atom, an alkyl group, an alkenyl group or an aryl group;  
 each  $R_2$  independently represents a halogen atom, an alkyl group, an alkenyl group, an alkoxy group, an aryl group, an aryloxy group, an alkylthio group, an arylthio group, an acyl group, an acylamino group, a sulfonyl group, a sulfonamide group or a hydroxy group;  
 each  $m$  is, individually an integer of 0 to 4; and  
 A represents an alkylene group having 1 to 6 carbon atoms in its linear structure.

The stabilizers that have the Formula R, above, are believed to stabilize the dye image by scavenging free radicals. In this formula, the group represented by A is a straight, branched, or cyclic alkylene group, the linear portion of which has 1 to 6 carbon atoms, which includes those such groups substituted with one or more aryl, cyano, halogen, heterocycl, cycloalkyl, alkoxy, hydroxy, and aryloxy groups. The alkylene group can form a cycloalkyl ring, such as



35

In Formula R, each  $R_1$  can be a group as defined above for  $R_6$  or  $R_7$  in Formula III. These include halogen, alkyl, cycloalkyl, alkenyl, alkoxy, aryl, aryloxy, alkylthio, arylthio, acyl, acylamino, sulfonyl and sulfonamido groups.

Preferred compounds represented by Formula R, are those in which:

- each  $R_1$  is independently hydrogen or a (cyclo)alkyl group of 1 to 8 carbon atoms;  
 each  $R_2$  is independently hydrogen, hydroxy, alkyl or alkoxy group of 1 to 8 carbon atoms;  
 each  $m$  is an integer of 0 to 2; and

A is an alkylene group of 1 to 10 carbon atoms.

Representative examples of stabilizer compounds which satisfy Formula R are:



R-1

60



R-2

55  
 65

-continued



R-3



R-4



R-5



R-6

35 The magenta dye forming couplers of this invention can be based on any of the bridgehead nitrogen 5,5 fused ring system identified above, Preferred couplers are pyrazolotriazoles represented by Formula II:

40 Formula II



wherein:

$R_6$  is hydrogen or a substituent;

$R_7$  is a ballast group or a fused benzene ring; and

X is hydrogen or a coupling-off-group; and

$Z_a$ ,  $Z_b$ , and  $Z_c$  are independently a substituted or unsubstituted methine group,  $=N-$ ,  $=C-$  or  $-NH-$ , provided that one of either the  $Z_a-Z_b$  bond or the  $Z_b-Z_c$  bond is a double bond and the other is a single bond, and when the  $Z_b-Z_c$  bond is a carbon-carbon double bond, it can be part of the aromatic ring and at least one of  $Z_a$ ,  $Z_b$ , and  $Z_c$  represents a methine group connected to  $R_7$ .

Preferred pyrazolotriazole couplers of this invention are 1H-pyrazolo[2,3-b][1,2,4]triazoles represented by Formula III:



Formula III

wherein:

X, R<sub>6</sub> and R<sub>7</sub> are as previously defined.

Examples of suitable R<sub>6</sub> groups are alkyl, which can be straight or branched, such as methyl, ethyl, n-propyl, n-butyl, t-butyl, trifluoromethyl, tridecyl or 3-(2,4-di-t-amylophenoxy)propyl; alkoxy, such as methoxy or ethoxy; alkylthio, such as methylthio or octylthio; aryl, aryloxy or arylthio, such as phenyl, 4-t-butylphenyl, 2,4,6-trimethylphenyl, phenoxy, 2- methylphenoxy, phenylthio or 2-butoxy-5-t-octylphenylthio; heterocyclyl, heterocyclyloxy or heterocyclthio, each of which contain a 3 to 7 membered heterocyclic ring composed of carbon atoms and at least one hetero atom selected from oxygen, nitrogen and sulfur, such as 2-furyl, 2-thienyl, 2-benzimidazolyloxy or 2-benzothiazolyl; cyano; acyloxy, such as acetoxy or hexadecanoyloxy; carbamoyloxy, such as N-phenylcarbamoyloxy or N-ethylcarbamoyloxy; silyloxy, such as trimethylsilyloxy; sulfonyloxy, such as dodecylsulfonyloxy; acylamino, such as acetamido or benzamido; anilino, such as phenylanilino or 2-chloroanilino; ureido, such as phenylureido or methylureido; imido, such as N-succinimido or 3-benzyihydantoinyl; sulfamoylamino, such as N,N-dipropyl-sulfamoylamino or N-methyl-N-decylsulfamoylamino; carbamoylamino, such as N-butylcarbamoylamino or N,N-dimethylcarbamoylamino; alkoxy carbonylamino, such as methoxycarbonylamino or tetradecyloxycarbonylamino; aryloxycarbonylamino, such as phenoxy carbonylamino, 2,4-di-t-butylphenoxy carbonylamino; sulfonamido, such as methanesulfonamido or hexadecanesulfonamido; carbamoyl group, such as N-ethylcarbamoyl or N,N-dibutylcarbamoyl; acyl, such as acetyl or (2,4-di-t-amylophenoxy)acetyl; sulfamoyl, such as N-ethylsulfamoyl or N,N-dipropylsulfamoyl; sulfonyl, such as methanesulfonyl or octanesulfonyl; sulfinyl, such as octanesulfinyl or dodecylsulfinyl; alkoxy carbonyl, such as methoxycarbonyl or butyloxycarbonyl; aryloxycarbonyl, such as phenoxy carbonyl

5 or 3-pentadecyloxycarbonyl; alkenyl; hydroxyl; amino; and carbonamido groups.  
Typically, R<sub>6</sub> represents a tertiary alkyl group of 4 to 12 carbon atoms, desirably, t-butyl.  
The ballast group represented by R<sub>7</sub> is a group of such size and configuration that, in combination with the remainder of the molecule, it provides the coupler, and the dye formed from it, with sufficient bulk that it is substantially non-diffusible from the layer in which it is coated in the photographic element. Representative ballast groups include alkyl or aryl groups containing 6 to 32 carbon atoms. Other ballast groups include alkoxy, aryloxy, arylthio, alkylthio, alkoxy carbonyl, aryloxycarbonyl, carboxy, acyl, acyloxy, carbonamido, carbamoyl, alkylcarbonyl, arylcarbonyl, alkylsulfonyl, arylsulfonyl, sulfamoyl, sulfenamoyl, alkylsulfinyl, arylsulfinyl, alkylphosphonyl, arylphosphonyl, alkylphosphonyl, alkoxyphosphonyl, and arylphosphonyl. Preferably R<sub>7</sub> is an alkyl group of 6 to 32 carbon atoms

10 Possible substituents for R<sub>6</sub> and R<sub>7</sub> include halogen, alkyl, aryl, aryloxy, heterocyclyl, cyano, alkoxy, acyloxy, carbamoyloxy, silyloxy, sulfonyloxy, acylamino, anilino, ureido, imido, sulfonylamino, carbamoylamino, alkylthio, arylthio, heterocyclthio, alkoxy carbonylamino, 20 aryloxycarbonylamino, sulfonamido, carbamoyl, acyl, sulfamoyl, sulfonyl, sulfinyl, alkoxy carbonyl, aryloxycarbonyl, alkenyl, carboxyl, sulfo, hydroxyl, amino and carbonamido groups.

25 The coupling off group represented by X can be a hydrogen atom or any of the coupling-off groups known in the art. Coupling-off groups can determine the equivalency of the coupler, can modify the reactivity of the coupler, or can advantageously affect the layer in which the coupler is coated or other layers in the element by performing, after the release from the coupler, such functions as development inhibition, development acceleration, bleach inhibition, bleach acceleration, color correction, and the like. Representative classes of coupling-off groups include halogen, particularly chlorine, bromine, or fluorine, alkoxy, aryloxy, heterocyclxy, heterocyclic, such as hydantoin and pyrazolo groups, sulfonyloxy, acyloxy, carbonamido, imido, acyl, heterocyclthio, sulfonamido, alkylthio, arylthio, heterocyclthio, sulfonamido, phosphonyloxy, and arylazo.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705

5,998,122

15

-continued

16

M-3



M-4



M-5



M-6



M-7



M-8



5,998,122

**17**

-continued

**18**

M-9



M-10



M-11



M-12



M-13



M-14



-continued

M-15



M-16



M-17



M-18



The couplers and compounds of the invention are readily manufactured as shown in the art and the synthetic example 35 herein. See U.S. Pat. Nos. 5,561,037; 5,236,819, and 4,124, 396. The elements of the invention provide useful photographic properties such as activity, hue, stability of coupler and dye, including light and dark keeping, as well as desirable processing characteristics such as process sensitivity.

Unless otherwise specifically stated, the term substituted or substituent means any group or atom other than hydrogen bonded to the remainder of a molecule. Additionally, when the term "group" is used, it means that when a substituent group contains a substitutable hydrogen, it is also intended to encompass not only the substituent's unsubstituted form, but also its form further substituted with any substituent group or groups as herein mentioned, so long as the substituent does not destroy properties necessary for photographic utility. Suitably, a substituent group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain or cyclic alkyl, such as methyl, trifluoromethyl, ethyl, t-butyl, 3-(2,4-di-t-pentylphenoxy) propyl, and tetradecyl; alkanyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy) ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradeccanamido, alpha-(2,4-di-t-pentyl-phenoxy)acetamido, alpha-(2,4-di-t-pentylphenoxy)

butyramido, alpha-(3-pentadecylphenoxy)-hexanamido, alpha-(4-hydroxy-3-t-butylphenoxy)-tetradecanamido, 35 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzoyloxycarbonylamino, hexadecyloxycarbonylamino, 40 2,4-di-t-butylphenoxy carbonylamino, phenyl carbonylamino, 2,5-(di-t-pentylphenyl) carbonylamino, p-dodecyl-phenyl carbonylamino, p-tolyl carbonylamino, N-methylureido, N,N-dimethylureido, N-methyl-N-dodecylureido, 45 N-hexadecylureido, N,N-di octadecylureido, N,N-di octyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and 50 t-butylcarbonamido; sulfonamido, such as methylsulfonamido, benzenesulfonamido, p-tolylsulfonamido, p-dodecylbenzenesulfonamido, N-methyltetradecylsulfonamido, N,N-dipropylsulfamoyl, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, 55 N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-di octylcarbamoyl; acyl, such as acetyl, (2,4-di-t-aminophenoxy)acetyl, phenoxy carbonyl, p-dodecyloxyphenoxy carbonyl, methoxycarbonyl, 60 butyoxycarbonyl, tetradecyloxycarbonyl, ethoxycarbonyl, benzoyloxycarbonyl, 3-pentadecyloxycarbonyl, and dodecyl-

loxcarbonyl; sulfonyl, such as methoxysulfonyl, octyloxysulfonyl, tetradecyloxysulfonyl, 2-ethylhexyloxysulfonyl, phenoxyulfonyl, 2,4-di-t-pentylphenoxyulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acetoxy, benzoxyloxy, octadecanoxyloxy, p-dodecylamidobenzoyloxy, N-phenylcarbamoyloxy, N-ethylcarbamoyloxy, and cyclohexylcarbonyloxy; amine, such as phenylanilino, 2-chloroanilino, diethylamine, dodecylamine; imino, such as 1-(N-phenylimido)ethyl, N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

The materials of the invention can be used in any of the ways and in any of the combinations known in the art. Typically, the invention materials are incorporated in a silver halide emulsion and the emulsion coated as a layer on a support to form part of a photographic element. Alternatively, unless provided otherwise, they can be incorporated at a location adjacent to the silver halide emulsion layer where, during development, they will be in reactive association with development products such as oxidized color developing agent. Thus, as used herein, the term "associated" signifies that the compound is in the silver halide emulsion layer or in an adjacent location where, during processing, it is capable of reacting with silver halide development products.

To control the migration of various components, it may be desirable to include a high molecular weight hydrophobe or "ballast" group in coupler molecules. Representative ballast groups include substituted or unsubstituted alkyl or aryl groups containing 8 to 48 carbon atoms. Representative substituents on such groups include alkyl, aryl, alkoxy, aryloxy, alkylthio, hydroxy, halogen, alkoxy carbonyl, aryloxy carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

If desired, the photographic element can be used in conjunction with an applied magnetic layer as described in *Research Disclosure*, November 1992, Item 34390 published by Kenneth Mason Publications, Ltd., Dudley Annex, 12a North Street, Emsworth, Hampshire P010 7DQ, ENGLAND, and as described in *Hatsumi Kyousai Koukai Gihou* No. 94-6023, published Mar. 15, 1994, available from the Japanese Patent Office, the contents of which are incorporated herein by reference. When it is desired to employ the inventive materials in a small format film, *Research Disclosure*, June 1994, Item 36230, provides suitable embodiments.

In the following discussion of suitable materials for use in the emulsions and elements of this invention, reference will be made to *Research Disclosure*, September 1996, Item 38957, available as described above, which is referred to herein by the term "Research Disclosure". The contents of the Research Disclosure, including the patents and publications referenced therein, are incorporated herein by reference, and the Sections hereafter referred to are Sections of the Research Disclosure.

Except as provided, the silver halide emulsion containing elements employed in this invention can be either negative-working or positive-working as indicated by the type of processing instructions (i.e. color negative, reversal, or direct positive processing) provided with the element. Suitable emulsions and their preparation as well as methods of chemical and spectral sensitization are described in Sections I through V. Various additives such as UV dyes, brighteners, antifoggants, stabilizers, light absorbing and scattering materials, and physical property modifying addenda such as hardeners, coating aids, plasticizers, lubricants and matting agents are described, for example, in Sections II and VI through VIII. Color materials are described in Sections X through XIII. Suitable methods for incorporating couplers and dyes, including dispersions in organic solvents, are described in Section X(E). Scan facilitating is described in Section XIV. Supports, exposure, development systems, and processing methods and agents are described in Sections XV to XX. The information contained in the September 1994 *Research Disclosure*, Item No. 36544 referenced above, is updated in the September 1996 *Research Disclosure*, Item No. 38957. Certain desirable photographic elements and processing steps, including those useful in conjunction with

color reflective prints, are described in Research Disclosure, Item 37038, February 1995.

Coupling-off groups are well known in the art. Such groups can determine the chemical equivalency of a coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction and the like.

The presence of hydrogen at the coupling site provides a 4-equivalent coupler, and the presence of another coupling-off group usually provides a 2-equivalent coupler. Representative classes of such coupling-off groups include, for example, chloro, alkoxy, aryloxy, hetero-oxy, sulfonyloxy, acyloxy, acyl, heterocycl, sulfonamido, mercaptotetrazole, benzothiazole, mercaptopropionic acid, phosphonyloxy, arylthio, and arylazo. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in UK Patents and published application Nos. 1,466,728, 1,531,927, 1,533,039, 2,006, 755A and 2,017,704A, the disclosures of which are incorporated herein by reference.

Image dye-forming couplers may be included in the element such as couplers that form cyan dyes upon reaction with oxidized color developing agents which are described in such representative patents and publications as: "Farbkuppler-eine Literature Ubersicht," published in Agfa Mitteilungen, Band III, pp. 156-175 (1961) as well as in U.S. Pat. Nos. 2,367,531; 2,423,730; 2,474,293; 2,772,162; 2,895,826; 3,002,836; 3,034,892; 3,041,236; 4,333,999; 4,746,602; 4,753,871; 4,770,988; 4,775,616; 4,818,667; 4,818,672; 4,822,729; 4,839,267; 4,840,883; 4,849,328; 4,865,961; 4,873,183; 4,883,746; 4,900,656; 4,904,575; 4,916,051; 4,921,783; 4,923,791; 4,950,585; 4,971,898; 4,990,436; 4,996,139; 5,008,180; 5,015,565; 5,011,765; 5,011,766; 5,017,467; 5,045,442; 5,051,347; 5,061,613; 5,071,737; 5,075,207; 5,091,297; 5,094,938; 5,104,783; 5,178,993; 5,813,729; 5,187,057; 5,192,651; 5,200,305; 5,202,224; 5,206,130; 5,208,141; 5,210,011; 5,215,871; 5,223,386; 5,227,287; 5,256,526; 5,258,270; 5,272,051; 5,306,610; 5,326,682; 5,366,856; 5,378,596; 5,380,638; 5,382,502; 5,384,236; 5,397,691; 5,415,990; 5,434,034; 5,441,863; EPO 0 246 616; EPO 0 250 201; EPO 0 271 323; EPO 0 295 632; EPO 0 307 927; EPO 0 333 185; EPO 0 378 898; EPO 0 389 817; EPO 0 487 111; EPO 0 488 248; EPO 0 539 034; EPO 0 545 300; EPO 0 556 700; EPO 0 556 777; EPO 0 556 858; EPO 0 569 979; EPO 0 608 133; EPO 0 636 936; EPO 0 651 286; EPO 0 690 344; German OLS 4,026,903; German OLS 3,624,777. and German OLS 3,823,049. Typically such couplers are phenols, naphthols, or pyrazoloazoles.

Couplers that form magenta dyes upon reaction with oxidized color developing agent are described in such representative patents and publications as: "Farbkuppler-eine Literature Ubersicht," published in Agfa Mitteilungen, Band III, pp. 126-156 (1961) as well as U.S. Pat.s Nos. 2,311,082 and 2,369,489; 2,343,701; 2,600,788; 2,908,573; 3,062,653; 3,152,896; 3,519,429; 3,758,309; 3,935,015; 4,540,654; 4,745,052; 4,762,775; 4,791,052; 4,812,576; 4,835,094; 4,840,877; 4,845,022; 4,853,319; 4,868,099; 4,865,960; 4,871,652; 4,876,182; 4,892,805; 4,900,657; 4,910,124; 4,914,013; 4,921,968; 4,929,540; 4,933,465; 4,942,116;

4,942,117; 4,942,118; 4,959,480; 4,968,594; 4,988,614; 4,992,361; 5,002,864; 5,021,325; 5,066,575; 5,068,171; 5,071,739; 5,100,772; 5,110,942; 5,116,990; 5,118,812; 5,134,059; 5,155,016; 5,183,728; 5,234,805; 5,235,058; 5,250,400; 5,254,446; 5,262,292; 5,300,407; 5,302,496; 5,336,593; 5,350,667; 5,395,968; 5,354,826; 5,358,829; 5,368,998; 5,378,587; 5,409,808; 5,411,841; 5,418,123; 5,424,179; EPO 0 257 854; EPO 0 284 240; EPO 0 341 204; EPO 0 347,235; EPO 0 365,252; EPO 0 422 595; EPO 0 428 899; EPO 0 428 902; EPO 0 459 331; EPO 0 467 327; EPO 0 476 949; EPO 0 487 081; EPO 0 489,333; EPO 0 512,304; EPO 0 515 128; EPO 0 534,703; EPO 0 554,778; EPO 0 558 145; EPO 0 571 959; EPO 0 583 832; EPO 0 583 834; EPO 0 584 793; EPO 0 602 748; EPO 0 602 749; EPO 0 605 918; EPO 0 622 672; EPO 0 622 673; EPO 0 629 912; EPO 0 646 841; EPO 0 656 561; EPO 0 660 177; EPO 0 686 872; WO 90/10253; WO 92/09010; WO 92/10788; WO 92/12464; WO 93/01523; WO 93/02392; WO 93/02393; WO 93/07534; UK Application 2,244,053; Japanese Application 03192-350; German OLS 3,624,103; German OLS 3,912,265; and German OLS 40 08 067. Typically such couplers are pyrazolones, pyrazoloazoles, or pyrazolobenzimidazoles that form magenta dyes upon reaction with oxidized color developing agents.

Couplers that form yellow dyes upon reaction with oxidized color developing agent are described in such representative patents and publications as: "Farbkuppler-eine Literature Ubersicht," published in Agfa Mitteilungen; Band III; pp. 112-126 (1961); as well as U.S. Pat. Nos. 2,298,443; 2,407,210; 2,875,057; 3,048,194; 3,265,506; 3,447,928; 4,022,620; 4,443,536; 4,758,501; 4,791,050; 4,824,771; 4,824,773; 4,855,222; 4,978,605; 4,992,360; 4,994,361; 5,021,333; 5,053,325; 5,066,574; 5,066,576; 5,100,773; 5,118,599; 5,143,823; 5,187,055; 5,190,848; 5,213,958; 5,215,877; 5,215,878; 5,217,857; 5,219,716; 5,238,803; 5,283,166; 5,294,531; 5,306,609; 5,328,818; 5,336,591; 5,338,654; 5,358,835; 5,358,838; 5,360,713; 5,362,617; 5,382,506; 5,389,504; 5,399,474; 5,405,737; 5,411,848; 5,427,898; EPO 0 327 976; EPO 0 296 793; EPO 0 365 282; EPO 0 379 309; EPO 0 415 375; EPO 0 437 818; EPO 0 447 969; EPO 0 542 463; EPO 0 568 037; EPO 0 568 196; EPO 0 568 777; EPO 0 570 006; EPO 0 573 761; EPO 0 608 956; EPO 0 608 957; and EPO 0 628 865. Such couplers are typically open chain ketomethylene compounds.

Couplers that form colorless products upon reaction with oxidized color developing agent are described in such representative patents as: UK. 861,138; U.S. Pat. Nos. 3,632,345; 3,928,041; 3,958,993 and 3,961,959. Typically such couplers are cyclic carbonyl containing compounds that form colorless products on reaction with an oxidized color developing agent.

Couplers that form black dyes upon reaction with oxidized color developing agent are described in such representative patents as U.S. Pat. Nos. 1,939,231; 2,181,944; 2,333,106; and 4,126,461; German OLS No. 2,644,194 and German OLS No. 2,650,764. Typically, such couplers are resorcinols or m-aminophenols that form black or neutral products on reaction with oxidized color developing agent.

In addition to the foregoing, so-called "universal" or "washout" couplers may be employed. These couplers do not contribute to image dye-formation. Thus, for example, a naphthol having an unsubstituted carbamoyl or one substituted with a low molecular weight substituent at the 2- or 3-position may be employed. Couplers of this type are described, for example, in U.S. Pat. Nos. 5,026,628, 5,151,343, and 5,234,800.

It may be useful to use a combination of couplers any of which may contain known ballasts or coupling-off groups

such as those described in U.S. Pat. Nos. 4,301,235; 4,853,319 and U.S. Pat. No. 4,351,897. The coupler may contain solubilizing groups such as described in U.S. Pat. No. 4,482,629. The coupler may also be used in association with "wrong" colored couplers (e.g. to adjust levels of interlayer correction) and, in color negative applications, with masking couplers such as those described in EP 213,490; Japanese Published Application 58-172,647; U.S. Pat. Nos. 2,983,608; 4,070,191; and 4,273,861; German Applications DE 2,706,117 and DE 2,643,965; UK. Patent 1,530,272; and Japanese Application 58-113935. The masking couplers may be shifted or blocked, if desired.

Typically, couplers are incorporated in a silver halide emulsion layer in a mole ratio to silver of 0.05 to 1.0 and generally 0.1 to 0.5. Usually the couplers are dispersed in a high-boiling organic solvent in a weight ratio of solvent to coupler of 0.1 to 10.0 and typically 0.1 to 2.0 although dispersions using no permanent coupler solvent are sometimes employed.

The invention materials may be used in association with materials that release Photographically Useful Groups (PUGS) that accelerate or otherwise modify the processing steps e.g. of bleaching or fixing to improve the quality of the image. Bleach accelerator releasing couplers such as those described in EP 193,389; EP 301,477; U.S. Pat. No. 4,163,669; 4,865,956; and U.S. Pat. No. 4,923,784, may be useful. Also contemplated is use of the compositions in association with nucleating agents, development accelerators or their precursors (UK Patent 2,097,140; UK. Patent 2,131,188); electron transfer agents (U.S. Pat. Nos. 4,859,578; 4,912,025); antifogging and anti color-mixing agents such as derivatives of hydroquinones, aminophenols, amines, gallic acid; catechol; ascorbic acid; hydrazides; sulfonamidophenols; and non color-forming couplers.

The invention materials may also be used in combination with filter dye layers comprising colloidal silver sol or yellow, cyan, and/or magenta filter dyes, either as oil-in-water dispersions, latex dispersions or as solid particle dispersions. Additionally, they may be used with "smearing" couplers (e.g. as described in U.S. Pat. No. 4,366,237; EP 96,570; U.S. Pat. No. 4,420,556; and U.S. Pat. No. 4,543,323.) Also, the compositions may be blocked or coated in protected form as described, for example, in Japanese Application 61/258,249 or U.S. Pat. No. 5,019,492.

The invention materials may further be used in combination with image-modifying compounds that release PUGS such as "Developer Inhibitor-Releasing" compounds (DIR's). DIR's useful in conjunction with the compositions of the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Color Photography,"

C. R. Barr, J. R. Thirtle and P. W. Vittum in *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzimidazoles, benzodiazoles, mercaptooxazoles, mercaptotriazoles, mercaptooxadiazoles, mercaptodiazoles, mercaptooxathiazoles, tellurotetrazoles or benzoisodiazoles. In a preferred embodiment, the inhibitor moiety or group is selected from the following formulas:



wherein R<sub>I</sub> is selected from the group consisting of straight and branched alkyls of from 1 to about 8 carbon atoms, 45 benzyl, phenyl, and alkoxy groups and such groups containing none, one or more than one such substituent; R<sub>II</sub> is selected from R<sub>I</sub> and —SR<sub>I</sub>; R<sub>III</sub> is a straight or branched alkyl group of from 1 to about 5 carbon atoms and m is from 1 to 3; and R<sub>IV</sub> is selected from the group consisting of 50 hydrogen, halogens and alkoxy, phenyl and carbonamido groups, —COOR<sub>V</sub> and —NHCOR<sub>V</sub> wherein R<sub>V</sub> is selected from substituted and unsubstituted alkyl and aryl groups.

Although it is typical that the coupler moiety included in the developer inhibitor-releasing coupler forms an image dye corresponding to the layer in which it is located, it may also form a different color as one associated with a different film layer. It may also be useful that the coupler moiety included in the developer inhibitor-releasing coupler forms 60 colorless products and/or products that wash out of the photographic material during processing (so-called "universal" couplers).

A compound such as a coupler may release a PUG directly upon reaction of the compound during processing, or indirectly through a timing or linking group. A timing group produces the time-delayed release of the PUG such groups using an intramolecular nucleophilic substitution reaction

## 27

(U.S. Pat. No. 4,248,962); groups utilizing an electron transfer reaction along a conjugated system (U.S. Pat. Nos. 4,409,323; 4,421,845; 4,861,701, Japanese Applications 57-188035; 58-98728; 58-209736; 58-209738); groups that function as a coupler or reducing agent after the coupler reaction (U.S. Pat. Nos. 4,438,193; 4,618,571) and groups that combine the features describe above. It is typical that the timing group is of one of the formulas:



wherein IN is the inhibitor moiety, R<sub>VII</sub> is selected from the group consisting of nitro, cyano, alkylsulfonyl; sulfamoyl; and sulfonamido groups; a is 0 or 1; and R<sub>VII</sub> is selected from the group consisting of substituted and unsubstituted alkyl and phenyl groups. The oxygen atom of each timing group is bonded to the coupling-off position of the respective coupler moiety of the DIAR.

The timing or linking groups may also function by 30 electron transfer down an unconjugated chain. Linking groups are known in the art under various names. Often they have been referred to as groups capable of utilizing a hemiacetal or iminoketal cleavage reaction or as groups capable of utilizing a cleavage reaction due to ester hydrolysis such as U.S. Pat. No. 4,546,073. This electron transfer down an unconjugated chain typically results in a relatively fast decomposition and the production of carbon dioxide, formaldehyde, or other low molecular weight by-products. The groups are exemplified in EP 464,612, EP 523,451, U.S. 40 Pat. No. 4,146,396, Japanese Kokai 60-249148 and 60-249149.

Suitable developer inhibitor-releasing couplers for use in the present invention include, but are not limited to, the following:



## 28

-continued

D2



D3



D4



D5



**29**

-continued

**30**

-continued

D9



D10



D11



D12



D6

5

10

15

D7

20

25

30

35

D8

40

50

55

60

65

It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire PO101 7DQ, England, incorporated herein by reference. Materials of the invention may be coated on pH adjusted support as described in U.S. Pat. No. 4,917,994; on a support with reduced oxygen permeability (EP 553,339); with epoxy solvents (EP 164,961); with nickel complex stabilizers (U.S. Pat. Nos. 4,346,165; 4,540,653 and U.S. Pat. No. 4,906,559 for example); with ballasted chelating agents such as those in U.S. Pat. No. 4,994,359 to reduce sensitivity to polyvalent cations such as calcium; and with stain reducing compounds such as described in U.S. Pat. No. 5,068,171. Other compounds useful in combination with the invention are disclosed in Japanese Published Applications described in Derwent Abstracts having accession numbers as follows: 90-072,629; 90-072,630; 90-072,631; 90-072,632; 90-072,633; 90-072,634; 90-077,822; 90-078,229; 90-078,230; 90-079,336; 90-079,337; 90-079,338; 90-079,690; 90-079,691; 90-080,487; 90-080,488; 90-080,489; 90-080,490; 90-080,491; 90-080,492; 90-080,494; 90-085,928; 90-086,669; 90-086,670; 90-087,360; 90-087,361; 90-087,362; 90-087,363; 90-087,364; 90-088,097; 90-093,662; 90-093,663; 90-093,664; 90-093,665; 90-093,666; 90-093,668; 90-094,055; 90-094,056; 90-103,409; 83-62,586; 83-09,959.

Conventional radiation-sensitive silver halide emulsions can be employed in the practice of this invention. Such emulsions are illustrated by *Research Disclosure*, Item 38755, September 1996, I. Emulsion grains and their preparation.

Especially useful in this invention are tabular grain silver halide emulsions. Tabular grains are those having two parallel major crystal faces and having an aspect ratio of at least 2. The term "aspect ratio" is the ratio of the equivalent circular diameter (ECD) of a grain major face divided by its thickness (t). Tabular grain emulsions are those in which the tabular grains account for at least 50 percent (preferably at least 70 percent and optimally at least 90 percent) of of total grain projected area. Preferred tabular grain emulsions are those in which the average thickness of the tabular grains is less than 0.3 micrometer (preferably thin—that is, less than 0.2 micrometer and most preferably ultrathin—that is, less than 0.07 micrometer). The major faces of the tabular grains can lie in either {111} or {100} crystal planes. The mean ECD of tabular grain emulsions rarely exceeds 10 micrometers and more typically is less than 5 micrometers.

In their most widely used form tabular grain emulsions are high bromide {111} tabular grain emulsions. Such emulsions are illustrated by Kofron et al U.S. Pat. No. 4,439,520, Wilgus et al U.S. Pat. No. 4,434,226, Solberg et al U.S. Pat. No. 4,433,048, Maskasky U.S. Pat. Nos. 4,435,501, 4,463,087 and 4,173,320, Daubendiek et al U.S. Pat. Nos. 4,414,310 and 4,914,014, Sowinski et al U.S. Pat. No. 4,656,122, Pigglin et al U.S. Pat. Nos. 5,061,616 and 5,061,609, Tsaur et al U.S. Pat. Nos. 5,147,771, '772, '773, 5,171,659 and 5,252,453, Black et al 5,219,720 and 5,334,495, Delton U.S. Pat. Nos. 5,310,644, 5,372,927 and 5,460,934, Wen U.S. Pat. No. 5,470,698, Fenton et al U.S. Pat. No. 5,476,760, Eshelman et al U.S. Pat. Nos. 5,612,175 and 5,614,359, and Irving et al U.S. Pat. No. 5,667,954.

Ultrathin high bromide {111} tabular grain emulsions are illustrated by Daubendiek et al U.S. Pat. Nos. 4,672,027, 4,693,964, 5,494,789, 5,503,971 and 5,576,168, Antoniades et al U.S. Pat. No. 5,250,403, Olm et al U.S. Pat. No.

5,503,970, Deaton et al U.S. Pat. No. 5,582,965, and Maskasky U.S. Pat. No. 5,667,955.

High bromide {100} tabular grain emulsions are illustrated by Mignot U.S. Pat. Nos. 4,386,156 and 5,386,156.

5 High chloride {111} tabular grain emulsions are illustrated by Wey U.S. Pat. No. 4,399,215, Wey et al U.S. Pat. No. 4,414,306, Maskasky U.S. Pat. Nos. 4,400,463, 4,713, 323, 5,061,617, 5,178,997, 5,183,732, 5,185,239, 5,399,478 and 5,411,852, and Maskasky et al U.S. Pat. Nos. 5,176,992 and 5,178,998. Ultrathin high chloride {111} tabular grain emulsions are illustrated by Maskasky U.S. Pat. Nos. 5,271,858 and 5,389,509.

High chloride {100} tabular grain emulsions are illustrated by Maskasky U.S. Pat. Nos. 5,264,337, 5,292,632, 5,275,930 and 5,399,477, House et al U.S. Pat. No. 5,320,938, Brust et al U.S. Pat. No. 5,314,798, Szajewski et al U.S. Pat. No. 5,356,764, Chang et al U.S. Pat. Nos. 5,413,904 and 5,663,041, Oyamada U.S. Pat. No. 5,593,821, Yamashita et al U.S. Pat. Nos. 5,641,620 and 5,652,088, Saitou et al U.S. Pat. No. 5,652,089, and Oyamada et al U.S. Pat. No. 5,665,530. Ultrathin high chloride {100} tabular grain emulsions can be prepared by nucleation in the presence of iodide, following the teaching of House et al and Chang et al, cited above.

25 The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is 30 conducted with uniform light exposure or in the presence of a nucleating agent. Tabular grain emulsions of the latter type are illustrated by Evans et al. U.S. Pat. No. 4,504,570.

35 Photographic elements can be exposed to actinic radiation, typically in the visible region of the spectrum, to form a latent image and can then be processed to form a visible dye image. Processing to form a visible dye image includes the step of contacting the element with a color developing agent to reduce developable silver halide and oxidize the color developing agent. Oxidized color developing agent in turn reacts with the coupler to yield a dye. If desired "Redox Amplification" as described in *Research Disclosure* XVIIIB(5) may be used.

40 With negative-working silver halide, the processing step described above provides a negative image. One type of such element, referred to as a color negative film, is designed for image capture. Speed (the sensitivity of the element to low light conditions) is usually critical to obtaining sufficient image in such elements. Such elements are typically silver bromoiodide emulsions coated on a transparent support and may be processed, for example, in known color negative processes such as the Kodak C-41 process as described in The British Journal of Photography Annual of 1988, pages 191-198. If a color negative film element is to be subsequently employed to generate a viewable projection print as for a motion picture, a process such as the Kodak ECN-2 process described in the H-24 Manual available from Eastman Kodak Co. may be employed to provide the color negative image on a transparent support. Color negative development times are typically 3'15" or less and desirably 90 or even 60 seconds or less.

45 The photographic element of the invention can be incorporated into exposure structures intended for repeated use or exposure structures intended for limited use, variously

33

referred to by names such as "single use cameras", "lens with film", or "photosensitive material package units".

Another type of color negative element is a color print. Such an element is designed to receive an image optically printed from an image capture color negative element. A 5 color print element may be provided on a reflective support for reflective viewing (e.g. a snap shot) or on a transparent support for projection viewing as in a motion picture. Elements destined for color reflection prints are provided on a reflective support, typically paper, employ silver chloride 10 emulsions, and may be optically printed using the so-called negative-positive process where the element is exposed to light through a color negative film which has been processed as described above. The element is sold with instructions to process using a color negative optical printing process, for 15 example the Kodak RA-4 process, as generally described in PCT WO 87/04534 or U.S. Pat. No. 4,975,357, to form a positive image. Color projection prints may be processed, for example, in accordance with the Kodak ECP-2 process as described in the H-24 Manual. Color print development times are typically 90 seconds or less and desirably 45 or even 30 seconds or less.

A reversal element is capable of forming a positive image without optical printing. To provide a positive (or reversal) image, the color development step is preceded by development with a non-chromogenic developing agent to develop exposed silver halide, but not form dye, and followed by uniformly fogging the element to render unexposed silver halide developable. Such reversal emulsions are typically sold with instructions to process using a color reversal 20 process such as the Kodak E-6 process as described in The British Journal of Photography Annual of 1988, page 194. Alternatively, a direct positive emulsion can be employed to obtain a positive image.

The above elements are typically sold with instructions to process using the appropriate method such as the mentioned color negative (Kodak C-41), color print (Kodak RA-4), or reversal (Kodak E-6) process.

Preferred color developing agents are p-phenylenediamines such as:

- 4-amino-N,N-diethylaniline hydrochloride,
- 4-amino-3-methyl-N,N-diethylaniline hydrochloride,
- 4-amino-3-methyl-N-ethyl-N-(2-methanesulfonamidoethyl)aniline sesquisulfate hydrate,
- 4-amino-3-methyl-N-ethyl-N-(2-hydroxyethyl)aniline sulfate,
- 4-amino-3-(2-methanesulfonamidoethyl)-N,N-diethylaniline hydrochloride, and
- 4-amino-N-ethyl-N-(2-methoxyethyl)-m-toluidine di-p-toluene sulfonic acid.

Development is usually followed by the conventional steps of bleaching, fixing, or bleach-fixing, to remove silver or silver halide, washing, and drying.

The entire contents of the patents and other publications referred to in this specification are incorporated herein by reference.

#### SYNTHETIC EXAMPLE

The following example illustrates the preparation of compounds of this invention. The purity of invention stabilizers were checked by (a) Thin Layer Chromatography in two or three different solvent systems of different polarity; (b) 300 MHz FT-NMR; (c) elemental analyses (C,H,N); and (d) mass spectral analysis.

34

The synthesis of Stabilizer 1-5 is given below:



A 5 L, 3n flask equipped with a mechanical stirrer, thermometer and a pressure equalized addition funnel was charged with commercially available ballast acid (356.2 g, 781.7 mol), THF (800 mL). The resulting amber solution was let stir under an Argon atmosphere. The addition funnel was charged with a solution of borane dimethyl sulfide complex, 2M in THF (1173 mL, 3 Eqs.). The borane dimethyl sulfide complex solution was added dropwise to the ballast acid solution. A slight exotherm was observed,  $T_1=27^\circ\text{ C}$ . to  $T_2=35^\circ\text{ C}$ . The reaction vessel was cooled in an ice bath to regulate the internal temperature to a constant  $30^\circ\text{ C}$ . throughout the addition period of 70 min. The reaction was let stir cooling to room temperature over night. An aliquot was removed and quenched into MeOH and mass spectral analysis showed (ES-) M-1=440 for desired product. The reaction vessel was cooled in a cold water bath and the addition funnel was charged with MeOH (500 mL) and was added dropwise over 1.5 hr and the resulting exotherm was controlled via cold water bath to an internal temperature of  $20^\circ\text{ C}$ . Another 500 mL was then added at room temperature, and the resulting solution was stirred overnight. The reaction solution was then stripped on a rotary evaporator, after which the residue was redissolved in MeOH (700 mL) and stripped; this process was then repeated. The residue was dissolved in EtOAc (1 L), transferred to a separatory funnel and washed with brine (3x350 mL), sat.  $\text{NH}_4\text{Cl}$  (1x350 mL), dried over  $\text{MgSO}_4$ , treated with decolorizing carbon, filtered and stripped to give 400 g of a clear oil which crystallized to a white solid on cooling. Solid was triturated with ligroin and collected and dried in a vacuum oven at  $30^\circ\text{ C}$ . for 24 hr to give 320.15 g (93% yield) of a white solid,  $\text{H}^1\text{ NMR}$  ( $\text{CDCl}_3$ ) which was consistent for desired structure, MS(ES-): M-1=440, mp.  $49\text{--}51^\circ\text{ C}$ . Further purification was required to remove residual sulfide. 316.45 g of stabilizer was dissolved in 1800 mL of  $\text{Et}_2\text{O}$ , solution was transferred to a 5 L separatory funnel and was washed with a 8%  $\text{H}_2\text{O}_2$  (3x325 mL), brine (1x500 mL), dried over  $\text{MgSO}_4$ , filtered through a pad of silica gel (6x15 cm), filtrate was concentrated on rotary evaporator to give a clear oil. The oil was dissolved in  $\text{Et}_2\text{O}$  (700 mL) and this solution was diluted with heptane to give a total volume of 3 L. This solution was seeded and chilled in ice to give I-5, as a white crystalline solid which was collected and washed with heptane. Solid was dried in a vacuum oven at  $30^\circ\text{ C}$ . for 24 h to give 294.0 g (93% recovery, 85% overall yield),  $\text{H}^1\text{ NMR}$  ( $\text{CDCl}_3$ ):  $\delta$  0.87 (q,  $J=7.0\text{ Hz}$ , 6H), 1.28 (s, 16H), 1.37 (m, 4H), 1.62 (m, 2H), 1.78 (m, 2H), 4.27 (m, 1H), 4.78 (br.s., 1H), 6.86 (d,  $J=1.8\text{ Hz}$ , 2H), 6.95 (s, 1H), 7.13 (d,  $J=1.8\text{ Hz}$ , 2H), MS(ES-): M-1=440, mp.  $49\text{--}51^\circ\text{ C}$ . Anal. Calcd. For  $\text{C}_{24}\text{H}_{43}\text{NO}_4\text{S}$ : C, 65.27; H, 9.80; N, 3.17. Found: C, 65.18; H, 9.71; N, 2.95.

## PHOTOGRAPHIC EXAMPLES

## Preparation of Photographic Elements

Coupler M-9 and coupler solvent diundecyl phthalate were dispersed in aqueous gelatin in the following manner:

Coupler M-9 (0.406 g,  $8.58 \times 10^{-4}$  mole) was dissolved in a mixture of diundecyl phthalate (0.686 g) and ethyl acetate (1.217 g). The mixture was heated to effect solution. After adding a solution of aqueous gelatin (21.82 g, 11.5%), diisopropylnaphthalene sulfonic acid (sodium salt) (2.51 g 10% solution), and water to make a total of 41.82 grams, the mixture was dispersed by passing it three times through a Gaulin homogenizer. This dispersion was used in the preparation of photographic element 101.

Dispersions containing the couplers and stabilizers shown for elements 102–114 in Table 1 were prepared in a similar manner. The amount of coupler in each dispersion was  $8.58 \times 10^{-4}$  mole, the amount of each stabilizer was as listed (in moles per mole coupler), and other components were the same as in Example 101. The photographic elements were prepared as follows: On a gel-subbed, polyethylene-coated paper support were coated the following layers:

## First Layer

An underlayer containing 3.23 grams gelatin per square meter.

## Second Layer

A photosensitive layer containing (per square meter) 2.15 grams total gelatin, an amount of green-sensitized silver chloride emulsion containing 0.172 grams silver; the dispersion containing  $5.38 \times 10^{-4}$  mole of the coupler indicated in Table 1; and 0.043 gram surfactant Alkanol XC (trademark of E.I. Dupont Co.) (in addition to the Alkanol XC used to prepare the coupler dispersion

## Third Layer

A protective layer containing (per square meter) 1.40 grams gelatin, 0.15 gram bis(vinylsulfonyl)methyl ether, 0.043 gram Alkanol XC, and  $4.40 \times 10^{-6}$  gram tetraethylammonium perfluorooctanesulfonate.

TABLE 1

| Element | Comparison or Invention | Coupler | Stabilizer(s) |
|---------|-------------------------|---------|---------------|
| 101     | Comparison              | M-9     | none          |
| 102     | Invention               | M-9     | I-3 (2.0)     |
| 103     | Invention               | M-9     | I-8 (2.0)     |
| 104     | Comparison              | M-9     | S-8 (0.5)     |
| 105     | Comparison              | M-9     | S-8 (0.5)     |
|         |                         |         | C-1 (2.0)     |
| 106     | Invention               | M-9     | S-8 (0.5)     |
|         |                         |         | I-3 (2.0)     |
| 107     | Invention               | M-9     | S-8 (0.5)     |
|         |                         |         | I-8 (2.0)     |
| 108     | Invention               | M-9     | S-8 (0.5)     |
|         |                         |         | I-6 (2.0)     |
| 109     | Invention               | M-9     | S-8 (0.5)     |
|         |                         |         | I-18 (2.0)    |
| 110     | Invention               | M-9     | S-8 (0.5)     |
|         |                         |         | I-19 (2.0)    |
| 111     | Comparison              | M-17    | S-8 (0.5)     |
| 112     | Invention               | M-17    | S-8 (0.5)     |
|         |                         |         | I-3 (2.0)     |
| 113     | Invention               | M-17    | S-8 (0.5)     |
|         |                         |         | I-8 (2.0)     |
| 114     | Comparison              | M-13    | S-8 (0.5)     |
| 115     | Invention               | M-13    | S-8 (0.5)     |
|         |                         |         | I-8 (2.0)     |
| 116     | Comparison              | M-16    | S-8 (0.5)     |
| 117     | Invention               | M-16    | S-8 (0.5)     |
|         |                         |         | I-8 (2.0)     |
| 118     | Comparison              | M-18    | S-8 (0.5)     |

TABLE 1-continued

| Element | Comparison or Invention | Coupler | Stabilizer(s)          |
|---------|-------------------------|---------|------------------------|
| 119     | Invention               | M-18    | S-8 (0.5)<br>I-8 (2.0) |

## Preparation of Processed Photographic Examples

Processed samples were prepared by exposing the coatings through a step wedge and processing as follows:

| Process Step | Time (min.) | Temp. (° C.) |
|--------------|-------------|--------------|
| Developer    | 0.75        | 35.0         |
| Bleach-Fix   | 0.75        | 35.0         |
| Water wash   | 1.50        | 35.0         |

The processing solutions used in the above process had the following compositions (amounts per liter of solution):

| Developer                                                                             |         |
|---------------------------------------------------------------------------------------|---------|
| Triethanolamine                                                                       | 12.41 g |
| Blankophor REU (trademark of Mobay Corp.)                                             | 2.30 g  |
| Lithium polystyrene sulfonate                                                         | 0.09 g  |
| N,N-Diethylhydroxylamine                                                              | 4.59 g  |
| Lithium sulfate                                                                       | 2.70 g  |
| 4-amino-3-methyl-N-ethyl-N-(2-methanesulfonamido ethyl)aniline sesquisulfate hydrate, | 5.00 g  |
| 1-Hydroxyethyl-1,1-diphosphonic acid                                                  | 0.49 g  |
| Potassium carbonate, anhydrous                                                        | 21.16 g |
| Potassium chloride                                                                    | 1.60 g  |
| Potassium bromide                                                                     | 7.00 mg |
| pH adjusted to 10.4 at 26.7 ° C.                                                      |         |
| Bleach-Fix                                                                            |         |
| Solution of ammonium thiosulfate                                                      | 71.85 g |
| Ammonium sulfite                                                                      | 5.10 g  |
| Sodium metabisulfite                                                                  | 10.00 g |
| Acetic acid                                                                           | 10.20 g |
| Ammonium ferric ethylenediaminetetraacetate                                           | 48.58 g |
| Ethylenediaminetetraacetic acid                                                       | 3.86 g  |
| pH adjusted to 6.7 at 26.7 ° C.                                                       |         |

The density of each step of each strip was measured. The maximum density of the strip in response to green light was recorded as "Dmax.". The strips were then covered by UV-absorbing filters (in lieu of coating a similar filter layer over the photosensitive layer of the photographic element) and subjected to irradiation by the light of a xenon arc lamp at an intensity of 50,000 lux for 2 weeks. The light stability of the dye ("Dye Stability"), expressed as the percent of the density remaining from initial densities of 1.0 and 1.7, is shown in Table 2.

TABLE 2

| Element | Comp/Inv   | Coup | Stab(s)   | Dye Stability-% remaining |          |          |
|---------|------------|------|-----------|---------------------------|----------|----------|
|         |            |      |           | Dmax                      | from 1.0 | from 1.7 |
| 101     | Comparison | M-9  | none      | 2.47                      | 16       | 31       |
| 102     | Invention  | M-9  | I-3       | 2.46                      | 71       | 75       |
| 103     | Invention  | M-9  | I-8       | 2.61                      | 77       | 80       |
| 104     | Comparison | M-9  | S-8       | 2.56                      | 69       | 74       |
| 105     | Invention  | M-9  | I-27      | 2.62                      | 75       | 79       |
| 106     | Comparison | M-9  | S-8       | 2.49                      | 70       | 75       |
| 107     | Comparison | M-9  | S-8 + C-1 | 2.74                      | 72       | 77       |
| 108     | Invention  | M-9  | S-8 + I-3 | 2.71                      | 83       | 86       |
| 109     | Invention  | M-9  | S-8 + I-8 | 2.70                      | 84       | 88       |

TABLE 2-continued

| Ele-<br>ment | Comp/Inv   | Coup | Stab(s)    | Dmax | Dye Stability-<br>% remaining<br>from 1.0 | Dye Stability-<br>% remaining<br>from 1.17 |
|--------------|------------|------|------------|------|-------------------------------------------|--------------------------------------------|
| 110          | Invention  | M-9  | S-8 + I-6  | 2.73 | 79                                        | 82                                         |
| 111          | Invention  | M-9  | S-8 + I-18 | 2.70 | 76                                        | 81                                         |
| 112          | Invention  | M-9  | S-8 + I-19 | 3.01 | 77                                        | 81                                         |
| 113          | Invention  | M-9  | S-8 + I-23 | 2.78 | 71                                        | 82                                         |
| 114          | Invention  | M-9  | S-8 + I-24 | 2.72 | 73                                        | 83                                         |
| 115          | Comparison | M-17 | S-8        | 2.15 | 83                                        | 82                                         |
| 116          | Invention  | M-17 | S-8 + I-3  | 2.61 | 84                                        | 86                                         |
| 117          | Invention  | M-17 | S-8 + I-8  | 2.68 | 87                                        | 89                                         |
| 118          | Comparison | M-13 | S-8        | 2.45 | 81                                        | 78                                         |
| 119          | Invention  | M-13 | S-8 + I-8  | 2.70 | 86                                        | 85                                         |
| 120          | Comparison | M-16 | S-8        | 2.00 | 95                                        | 94                                         |
| 121          | Invention  | M-16 | S-8 + I-8  | 2.64 | 98                                        | 98                                         |
| 122          | Comparison | M-18 | S-8        | 3.00 | 84                                        | 86                                         |
| 123          | Invention  | M-18 | S-8 + I-8  | 3.22 | 92                                        | 91                                         |

It is clear from the data in Table 1 that the stabilizers of our invention provided substantial improvements in the light stability of the magenta image dye when used in the absence of any additional stabilizers (Examples 102–103 vs. Example 101).

The data also show that the stabilizers of the invention provided substantial improvements in the light stability of the magenta image dye when used in combination with the known stabilizer Compound S-8 (Examples 107–114 vs Example 106, and Examples 116–117 vs Example 115). Comparison stabilizer C-1 is a hydroxylalkyl compound but lacks the other required structural features of formula I, provided only slightly better stabilization in combination with S-8 than S-8 alone (Example 105 vs Example 104).

Examples 118–123 show that the stabilizers of our invention are effective with a wide range of different types of couplers that are within the scope of the invention.

Stabilizer I-27, which combines the functionalities of formula I with those of formula S, provided better light stability than Compound S-8, which lacks several of the structural features of formula I (Example 105 vs Example 104).

The data in Table 2 also show that in nearly every comparison, the elements containing the stabilizers of our invention provided significant boosts in the density of the dye formed during color development, represented by Dmax, compared to the corresponding elements that did not contain the stabilizers of our invention.

The invention has been described in detail with particular reference to certain preferred embodiments thereof, but it will be understood that variations and modifications can be effected within the spirit and scope of the invention.

What is claimed is:

1. A photographic element comprising a light sensitive silver halide emulsion layer having associated therewith a magenta dye forming coupler containing an azole nucleus and a ballasted compound having Formula I,



wherein

each R<sub>1</sub> is independently selected from the group consisting of hydrogen and an alkyl, aryl, acyl and acylamino group;

I

60

wherein:

each R<sub>1</sub> independently represents a hydrogen atom, an alkyl group, an alkenyl group or an aryl group; each R<sub>2</sub> independently represents a substituent; each m independently represents an integer of 0 to 4; and A represents an alkylene group having 1 to 6 carbon atoms in its linear structure.

5. A photographic element of claim 4 wherein compound S has the structure:



wherein:

R<sub>3</sub> represents an aryl group or a heterocyclic group; Z<sub>1</sub> and Z<sub>2</sub> each represent an alkylene group having 1 to 3 carbon atoms provided that the total number of carbon atoms in the ring is 3 to 6;

n is an integer of 1 or 2.

3. A photographic element of claim 1, wherein said silver halide emulsion layer has associated therewith a compound having Formula R:



wherein:

each R<sub>1</sub> independently represents a hydrogen atom, an alkyl group, an alkenyl group or an aryl group; each R<sub>2</sub> independently represents a substituent; each m independently represents an integer of 0 to 4; and A represents an alkylene group having 1 to 6 carbon atoms in its linear structure.

4. A photographic element of claim 2, wherein said silver halide emulsion layer has associated therewith a compound having Formula R:



wherein:

each R<sub>1</sub> independently represents a hydrogen atom, an alkyl group, an alkenyl group or an aryl group; each R<sub>2</sub> independently represents a substituent; each m independently represents an integer of 0 to 4; and A represents an alkylene group having 1 to 6 carbon atoms in its linear structure.



wherein:

R<sub>8</sub> represents halogen or an alkyl, alkoxy, alkylthio, amido, or ureido group;  
R<sub>9</sub> is an alkyl group;  
r is an integer of 1 or 2; and  
s is an integer of 0 to 4; and  
compound R has the structure:



wherein

each R<sub>1</sub> independently represents hydrogen, alkyl or cycloalkyl groups of 1 to 8 carbon atoms;  
each R<sub>2</sub> is independently hydrogen, hydroxy, alkyl or alkoxy of 1 to 8 carbon atoms;  
each m is an integers of 0 to 2; and  
A is an alkylene group of 1 to 10 carbon atoms.

6. A photographic element of claim 4, wherein each of compounds S, I and R are associated with said silver halide emulsion layer in an amount in a range of about 0.2 to 2.0 moles compound per mole magenta dye forming coupler.

7. A photographic element of claim 1, said silver halide emulsion layer further having associated therewith a phthalate ester coupler solvent.

8. A photographic element of claim 1, wherein the magenta dye forming coupler has the structure:



Formula II 40

wherein:

R<sub>6</sub> is hydrogen or a substituent;  
R<sub>7</sub> is a ballast group or a fused benzene ring; and  
X is hydrogen or a coupling-off-group; and  
Z<sub>a</sub>, Z<sub>b</sub>, and Z<sub>c</sub> are independently a substituted or unsubstituted methine group, =N—, =C— or —NH—, provided one of either the Z<sub>a</sub>—Z<sub>b</sub> bond or the Z<sub>b</sub>—Z<sub>c</sub> bond is a double bond and the other is a single bond, and when the Z<sub>b</sub>—Z<sub>c</sub> bond is a carbon-carbon double bond, it can be part of the aromatic ring and at least one of Z<sub>a</sub>, Z<sub>b</sub>, and Z<sub>c</sub> represents a methine group connected to R<sub>7</sub>.

9. A photographic element of claim 4, wherein the magenta dye forming coupler has the structure:



Formula III

wherein:

R<sub>6</sub> is hydrogen or a substituent;

R<sub>7</sub> is a ballast group; and

X is hydrogen or a coupling-off-group.

10. A photographic element of claim 4, wherein R<sub>6</sub> is a tertiary alkyl group.

11. A photographic element of claim 1, wherein compound I has the structure:



wherein:

R<sub>1</sub> and R<sub>2</sub> are alkyl groups having a total of 9-30 carbon atoms.

12. Photographic element of claim 1, wherein I has the structure:



I-8

13. A photographic element of claim 1 wherein the support is opaque.

14. A photographic element of claim 1 wherein the coupler and compound I are directly dispersed in said silver halide emulsion without the use of a coupler solvent.

15. A photographic element of claim 1 that is suitable for direct viewing after development.

16. A photographic element of claim 1 wherein said silver halide emulsion comprises at least 90 mole percent silver chloride.

17. A photographic element of claim 8 wherein R<sub>7</sub> is a fused benzene ring group.